

# United States Patent [19]

Minagawa

[11] 3,787,214

[45] Jan. 22, 1974

[54] PROCESS FOR UNDERCOATING A SUPPORT OF PHOTOGRAPHIC MATERIAL

[75] Inventor: Nobuhiko Minagawa, Fujinomiya, Japan

[73] Assignee: Fuji Photo Film Co., Ltd., Minami Ashigara-shi, Kanagawa, Japan

[22] Filed: Sept. 24, 1971

[21] Appl. No.: 183,656

[30] Foreign Application Priority Data

Sept. 24, 1970 Japan..... 45-83649

[52] U.S. Cl..... 96/87 R, 96/85, 117/34,

117/47 A

[51] Int. Cl..... G03c 1/80, G03c 1/86

[58] Field of Search ..... 96/85, 87 R; 117/47 A, 34

[56] References Cited

UNITED STATES PATENTS

3,320,191 5/1967 Secrist..... 96/87 R

3,161,519 12/1964 Alsup..... 96/85  
3,123,492 3/1964 Maffet..... 96/87 R

## FOREIGN PATENTS OR APPLICATIONS

1,134,211 11/1964 Great Britain..... 96/85

*Primary Examiner*—Ronald H. Smith  
*Attorney, Agent, or Firm*—Richard C. Sughrue et al.

[57] ABSTRACT

A process for undercoating a support of a photographic material is disclosed comprising providing an undercoat layer containing gelatin and a basic substance, such as sodium hydroxide, on an activated surface of a support comprising a polyolefin film or a polyolefin-coated film, said basic substance being included therein so as to maintain the hydrogen ion concentration (pH) of the surface of the undercoat layer at a level of from 6.6 to 9.5. A photographic emulsion adheres firmly to the undercoated surface of the support with a markedly increased bond strength.

7 Claims, No Drawings

# PROCESS FOR UNDERCOATING A SUPPORT OF PHOTOGRAPHIC MATERIAL

## BACKGROUND OF THE INVENTION

### 1. Field of the Invention

This invention relates to a process for undercoating a photographic material support composed of a polyolefin film or a polyolefin-coated film.

### 2. Description of the Prior Art

A polyolefin surface is chemically inert, and therefore, when a photographic emulsion is directly coated on such a surface, the support does not adhere at all to the photographic emulsion layer. Accordingly, it has previously been the practice to subject such a polyolefin surface to an activating treatment such as a corona-discharge treatment, or a flame treatment, before applying a photographic emulsion layer to the surface.

Furthermore, in order to prevent the deterioration of the activating treatment effect with the passage of time before the application of a photographic emulsion, undercoating of the activated polyolefin surface with a hydrophilic resin has previously been performed.

However, neither the activating treatment nor the undercoating after the activating treatment has given a practically satisfactory bond strength between the support and the photographic emulsion layer.

Extensive work on undercoating methods in an attempt to remove these defects of the prior art has finally led to the accomplishment of the present invention.

## SUMMARY OF THE INVENTION

According to the present invention, there is provided a process for undercoating a support of a photographic material, which comprises providing an undercoating of gelatin on the activated surface of a support having a polyolefin surface, and maintaining the hydrogen ion concentration (to be abbreviated as pH hereinafter) of the surface of the undercoat layer at from 6.6 to 9.5, whereby the bond strength between the support and a layer of a photographic emulsion is exceedingly increased.

## DESCRIPTION OF THE PREFERRED EMBODIMENTS:

The support used in this invention is a polyolefin film or a polyolefin-coated film obtained by coating at least one surface of a support made of a material such as paper, cellophane, cellulose acetate or polyester, with a polyolefin. By the term "polyolefin", as used in the present specification, is meant polyethylene, polypropylene or mixtures thereof. The polyolefin film is obtained by an ordinary film-forming method such as the tubular film method, or flat die method. The polyolefin-coated film is obtained by the extrusion coating method or the adhering method using an adhesive.

The undercoat layer in the present invention consists essentially of gelatin. The undercoat layer is prepared by coating an aqueous solution of gelatin or a dispersion of an aqueous gelatin solution in an organic solvent compatible with water, onto the surface of a polyolefin support which has been subjected to the activating treatment. The gelatin solution preferably has a concentration of from 0.1 to 15 percent by weight.

Suitable activating treatments, known to those skilled in the art, can be employed depending on the charac-

teristics desired. An example of a suitable activating treatment is disclosed in "Tappi," Volume 48, No. 9; September, 1965; pp. 80-84.

The pH adjustment of the surface of the undercoat layer is effected by adding any water-soluble hydrophilic basic substance to the under-coat solution. Examples of typical basic substances include sodium hydroxide, potassium hydroxide, sodium carbonate, and sodium bicarbonate, although it is to be expressly understood that any hydrophilic basic substance which performs the function of adjusting the pH to from 6.6 to 9.5, is operable.

The polyolefin film or coating of the support preferably has a thickness of from about 10 to 100 microns and the undercoat layer preferably has a thickness of from about 0.01 to 10 microns.

In addition, if desired, the undercoat layer can have incorporated therein up to about 30 percent by weight of a low molecular weight carboxylic acid, such as, for example, formic acid, propionic acid, acrylic acid or salicylic acid. The acid is added to the layer in order to stabilize the colloidal gelatin in the non-soluble liquid medium.

The measurement of the pH of the undercoat surface was made by a color test using a litmus solution and a color test using a paper surface pH measuring solution (product of Kabushiki Kaisha Kyoritsu Rikagaku Kenkyusho).

The bond strength between the support and the photographic emulsion layer was measured as follows:

### 1. Bond strength in a dry state after or before the photographic processing:

Checkerboard like, criss-crossing lines (the space between the lines being about 4 mm) were provided on the emulsion surface of the support using a razor blade. An adhesive tape was applied to it from above, and then peeled off quickly. When more than 90 percent of the emulsion surface remained unpeeled, the bond strength was evaluated as good.

### 2. Bond strength in a processing solution:

One scratch, i.e., score, was made on the emulsion surface while the material was immersed in a processing solution using a stylus, and the injured, i.e., scored, portion was rubbed with a finger tip at right angles to the injury. When the photographic emulsion layer did not come off more than the injury, the bond strength was evaluated as good.

In tests with the photographic material using the support and undercoat layer of the present invention, the bond strength between the support and the photographic emulsion layer was always evaluated as good.

The invention will now be described specifically by the following Examples which are presented for illustrative, rather than limitative purposes.

## EXAMPLE 1

Polyethylene having a density of 0.92 g/cm<sup>3</sup> was extrusion-coated onto both surfaces of a photographic raw paper having a unit weight of 150 g/m<sup>2</sup> in a thickness of about 30 microns. One surface of the polyethylene-coated paper onto which a photographic emulsion was to be coated was subjected to a corona discharge treatment using a corona discharge apparatus having a movable electrode and disposed at a position 0.8 mm away from said surface. The discharge output per unit length of the electrode was 10 W/cm, and the electrode

moving speed of 20 m/min. Thereafter, each under-coating solution of the following formulations, Nos. 1 and 2, was coated on to separate samples, each having the treated surface as described above, and dried.

## Formulation No. 1

Gelatin 50 g  
Water 400 cc  
Methanol 600 cc

## Formulation No. 2.

## Formulation No. 4:

Gelatin 50 g  
Salicylic acid 5 g  
Sodium carbonate 1.6 g  
Water 300 cc  
Methanol 700 cc

A gelatin-silver halide emulsion was coated onto each sample's undercoated surface of the polypropylene film, and the bond strength between the support and the photographic emulsion layer was measured, and the results are shown in Table 2.

Table 2

| Formulation of the under-coating solution | pH values of the under-coated surface | Bond strength                                     |                                                        |
|-------------------------------------------|---------------------------------------|---------------------------------------------------|--------------------------------------------------------|
|                                           |                                       | Dry state (percentage of unpeeled emulsion layer) | Wet state (maximum width of the peeled emulsion layer) |
| No. 3                                     | 5.2                                   | 70 - 75%                                          | 15 - 20 mm                                             |
| No. 4                                     | 6.8                                   | 90 - 100%                                         | 0 mm                                                   |

Gelatin 50 g  
Sodium hydroxide 0.4 g  
Water 400 cc  
Methanol 600 cc

The undercoated surfaces of each polyethylene-coated paper were coated with an ordinary photographic emulsion.

The bond strength between the support and the emulsion layer of each of the resultant water-resistant photographic papers was measured, and the results are shown in Table 1. The pH values of the undercoated surfaces of the polyethylene-coated papers are also shown in Table 1.

Different portions of one surface of a high density polyethylene film having a thickness of 150 microns, onto which a photographic emulsion was to be coated, were subjected to a corona discharge treatment using a corona discharge apparatus of the type shown in Example 1, and then immediately coated with separate undercoating solutions of the formulations Nos. 5 and 6.

## Formulation No. 5:

Gelatin 75 g  
Salicylic acid 7.5 g

Table 1

| Formulation of the under-coating solution | pH values of the under-coated surface | Bond Strength                                     |                                                        |
|-------------------------------------------|---------------------------------------|---------------------------------------------------|--------------------------------------------------------|
|                                           |                                       | Dry state (percentage of unpeeled emulsion layer) | Wet state (maximum width of the peeled emulsion layer) |
| No. 1                                     | 6.2                                   | 75-85%                                            | 2 - 3 mm                                               |
| No. 2                                     | 6.6                                   | 95-100%                                           | 0 mm                                                   |

## EXAMPLE 2

Different portions of one surface of a crystalline polypropylene film having a thickness of 150 microns were flame treated with a gaseous mixture of propane and oxygen, and then immediately coated with separate undercoating solutions, each of the following formulations, Nos. 3 and 4, followed by drying.

## Formulation No. 3:

Gelatin 50 g  
Salicylic acid 5 g  
Water 300 cc  
Methanol 700 cc

Water 300 cc  
Methanol 700 cc

## Formulation No. 6:

Gelatin 75 g  
Salicylic acid 7.5 g  
Potassium hydroxide 5 g  
Water 300 cc  
Methanol 700 cc

A gelatin-silver halide emulsion was coated onto each sample's undercoated surface of the polyethylene film. The bond strength between the support and the emulsion layer of the resultant photographic materials was measured, and the results are shown in Table 3.

Table 3

| Formulation<br>of the under-<br>coating<br>solution | pH values of<br>the under-<br>coated<br>surface | Bond strength                                                |                                                                 |
|-----------------------------------------------------|-------------------------------------------------|--------------------------------------------------------------|-----------------------------------------------------------------|
|                                                     |                                                 | Dry state<br>(percentage of<br>unpeeled emul-<br>sion layer) | Wet state<br>(maximum width<br>of the peeled<br>emulsion layer) |
| No. 5                                               | 5.2                                             | 70 - 75%                                                     | 15 - 20 mm                                                      |
| No. 6                                               | 9.5                                             | 95 - 100%                                                    | 0 mm                                                            |

## What is claimed is:

1. A photographic material comprising a support selected from the group consisting of a polyolefin support and a polyolefin-coated support, the surface of said support being activated, having coated thereon an undercoat layer consisting essentially of gelatin and a hydrophilic basic substance present in an amount sufficient to provide the surface of the undercoat layer with a pH of from 6.6 to 9.5 and a photographic emulsion coated onto said undercoat layer.

2. The photographic material of claim 1 wherein the polyolefin is polyethylene, polypropylene or a mixture thereof.

3. The photographic material of claim 2, wherein the basic substance is sodium hydroxide, potassium hydroxide, sodium carbonate or sodium bicarbonate.

4. The photographic material of claim 2 wherein said undercoat layer further comprises up to about 30 weight percent of a low molecular weight carboxylic acid.

5. The photographic material of claim 1, wherein the thickness of said undercoat layer is from about 0.01 to 10 microns.

6. The photographic material of claim 1 wherein the polyolefin portion of said support is from 10 to 100 microns in thickness.

7. A process for producing a photographic material comprising providing an undercoat layer consisting essentially of gelatin and a hydrophilic basic substance on an activated surface of a support selected from the group consisting of a polyolefin support and a polyolefin-coated support, said hydrophilic basic substance being included to maintain the pH of the surface of the undercoat layer at a level of from 6.6 to 9.5, and coating a photographic light-sensitive emulsion onto said undercoat layer.

\* \* \* \* \*

30

35

40

45

50

55

60

65